

# United States Patent [19]

Amati et al.

[11] 3,821,023

[45] June 28, 1974

[54] **CREASE RESISTANT FINISH FOR TEXTILES HAVING IMPROVED SOIL REPELLENT PROPERTIES**

[75] Inventors: Werner Amati, Pratteln/Bl; Richard Hochreuter, Oberwil/Bl, both of Switzerland

[73] Assignee: Sandoz Ltd., Basel, Switzerland

[22] Filed: Dec. 20, 1971

[21] Appl. No.: 210,116

[30] **Foreign Application Priority Data**

Dec. 22, 1970 Switzerland..... 18949/70

[52] U.S. Cl. 117/139.5 A, 117/138.8 F, 117/139.4, 117/143 R

[51] Int. Cl. .... C08j 1/44

[58] Field of Search ..... 117/139.5 CQ, 139.5 R, 117/139.5 A, 138.8 F, 138.8 B, 143 R, 139.4; 252/8.6; 260/470

[56] **References Cited**

UNITED STATES PATENTS

|           |         |                       |              |
|-----------|---------|-----------------------|--------------|
| 1,935,264 | 11/1933 | Felix .....           | 260/470      |
| 2,917,412 | 12/1959 | Reinhardt et al. .... | 117/139.4 UX |
| 3,144,299 | 8/1964  | Frick et al. ....     | 117/139.4    |

Primary Examiner—William D. Martin

Assistant Examiner—Theodore G. Davis

Attorney, Agent, or Firm—Gerald D. Sharkin; Richard E. Vila; Thomas C. Doyle

## ABSTRACT

Compounds for the soil repellent finishing of textiles of the general formula



wherein

R stands for a p-valent radical of an organic compound which has one to 40 carbon atoms and contains at least one active hydrogen atom,

R' for hydrogen or for a saturated or unsaturated alkyl or an aromatic radical or an aliphatic carboxylic acid radical which has one to 30 carbon atoms or for the radical of an inorganic acid which may be esterified,

m for the value 2, 3 or 4,

n for zero or a value from 1 to 100,

y for zero or the value 1,

p for a value from 1 to 4

X for -NH- or -N-Z where Z is a lower alkyl radical which may be substituted;

and where the molecule has a minimum molecular weight of 100 and bears at least one free acid group are applied to textiles in conjunction with a crease-proofing N-methylol resin and a catalyst for the resin.

14 Claims, No Drawings

**CREASE RESISTANT FINISH FOR TEXTILES  
HAVING IMPROVED SOIL REPELLENT  
PROPERTIES**

As is known, textiles of the various synthetic and cellulosic fibres, alone or in blends, in particular polyester fibre textiles, which have been finished with N-methylol resins, show enhanced power of soil retention which means that they become heavily soiled in use and when washed cannot readily be cleared of the impurities.

In order to overcome or diminish this undesirable behaviour, textiles of these fibres are finished with hydrophilic compounds. The products which have found acceptance in the textile industry for this purpose include the polyacrylic acid derivatives disclosed in U.S. Pat. No. 3,377,249, the polyoxyalkylene glycol terephthalic acid copolymers disclosed in French Pat. No. 1,502,969, the monostearic acid polyglycol esters disclosed in British Pat. No. 738,379 and the adducts of ethylene oxide and propylene oxide on alkyl phenols which are described in the published Swiss Pat. application 6149/68 and the published German Pat. application 1,914,389.

These products all have certain disadvantages. The polyacrylic acid derivatives impart a harsh, stiff handle to the finished fabric, the polyoxyalkylene glycol terephthalic acid copolymers are not applicable to cotton, while the monostearic acid-polyglycol esters, and the ethylene oxide and propylene oxide adducts on alkyl phenols leave the fabric with unsatisfactory wash resistance and impair the fastness properties of dyed goods, especially if they have been dyed with disperse dyes.

It has been found that these disadvantages are absent when compounds of formula (I) below are used for the soil repellent finishing of textiles, in combination with a resin, for example one of the resins used for crease resistant finishing, while the soil repellency thereby obtained is greater than that given by the aforesaid compounds.

This invention therefore relates to the use for the soil repellent finishing of textile fibres, yarns and fabrics of compounds agreeing with the general formula



where

R stands for a p-valent radical of an organic compound which has one to 40 carbon atoms and contains at least one active hydrogen atom,

R' for hydrogen or for a saturated or unsaturated alkyl or an aromatic radical or an aliphatic carboxylic acid radical which has 1 to 30 carbon atoms or for the radical of an inorganic acid which may be esterified,

n for the value 2, 3 or 4,

y for zero or a value from 1 to 100,

p for zero or the value 1,

p for a value from 1 to 4

X for -NH- or



where Z is a lower alkyl radical which may be substituted;

and where the molecule has a minimum molecular weight of 100 and bears at least one free acid group.

The p-valent radical R is the radical of a compound R(H)<sub>p</sub> having at least p active hydrogen atoms, which may be present in the form of hydroxyl (-OH) groups or



groupings. These may be bound to a carbon atom either directly or through a sulphur or phosphorus atom. The active hydrogen in the compound R(H)<sub>p</sub> can thus be an alcohol or thioalcohol group or an acid group, occurring for example as a -COOH, -SO<sub>3</sub>H, SO<sub>2</sub>H, -PO<sub>3</sub>H<sub>2</sub> or -PO<sub>2</sub>H<sub>2</sub> group or as an amide grouping such as



bound on a carbon atom. Alternatively, the -OH group or -NH grouping may be bound to a partially esterified acid group, for example -PO<sub>2</sub>(L)OH, where the preferred meaning of L is that of an optionally substituted alkyl or alkenyl radical having one to 30 carbon atoms.

The p-valent radical R consists of an optionally further unsubstituted or substituted alkyl, alkenyl or aromatic radical having one to 40 carbon atoms, these atoms bearing at least one of the aforesaid alcoholic, thioalcoholic, acid or amidated groups which is capable of binding an active hydrogen atom. The preferred unsubstituted or substituted alkyl radicals have one to 40 carbon atoms, special preference being given to aliphatic hydrocarbon radicals with two to 22 carbon atoms which may bear aromatic ring systems as substituents. The substituents on the alkyl radicals are preferably phenyl, naphthyl, diphenyl, diphenylether, diphenylsulphide or diphenylmethane radicals, which may be further substituted by hydroxyl, lower alkyl or an acid radical.

Besides the distinctive feature of being monomeric in character and bearing at least one free acid group, the disclosed compounds are further characterized by the fact that the value of n may vary within wide limits. Compounds with high n values are of major interest for the finishing of white goods. In these, the introduction of several free acid groups, in particular carboxymethyl groups or phosphorus or sulphonic acid groups which may if desired by esterified, has a favourable effect. Given low n values, it is of advantage to introduce hydrocarbon radicals of high molecular weight.

Notably good results are obtained when the following R radicals are employed:





$\text{C}_{18}\text{H}_{35}\text{O}-$ ,  $\text{C}_{11}\text{H}_{23}\text{COO}-$ ,  $\text{C}_{17}\text{H}_{35}\text{COO}-$ ,  $\text{C}_{15}\text{H}_{33}\text{O}-$ ,  
or  $\text{C}_{17}\text{H}_{33}\text{COO}-$

The radicals  $\text{-C}_8\text{H}_{17}$ ,  $\text{-C}_{18}\text{H}_{35}$ ,



$\text{-C}_6\text{H}_4\text{C}_9\text{H}_{19}$ ,  $\text{-SO}_3\text{H}$ ,  $\text{-PO}_3\text{H}_2$  and  $\text{-CH}_2\text{COONa}$  and also 30 the homologous series of  $\text{C}_8\text{H}_{17}$  to  $\text{C}_{18}\text{H}_{35}$  radicals are highly suitable as  $\text{R}'$  radicals, and given certain conditions those named as meanings of  $\text{R}$  are also of interest.

The compounds of this invention contain at least one 35 but preferably not more than five free acid groups, which may be present as alkali-metal or ammonium salts. Optimally one to three acid groups are present.

The compound of formula I should have a minimum molecular weight of 100.

The compounds employed in accordance with this invention can be produced by known methods or in analogy with known methods, with the necessary condition that one free acid group remains in the reaction product or is introduced into it. A number of these methods are outlined below.

a. Reaction of a sulphonated or unsulphonated aliphatic or aromatic carboxylic acid or a carboxylic acid derivative with an aliphatic alcohol or with an alkyl, aryl or alkylaryl polyglycoether at elevated temperature.

b. Esterification of an unsaturated monocarboxylic or polycarboxylic acid or a derivative of such an acid with an alcohol or with alkyl, aryl or alkylaryl polyglycol ether at high temperature, if necessary with the aid of a catalyst, with subsequent addition of e.g. sodium sulphite or sodium hydrosulphite in aqueous solution.

c. Reaction of a polycarboxylic anhydride with an aliphatic alcohol or an amine and subsequent esterification of a carboxylic acid group with a polyglycol in the presence of catalyst to yield the diester.

d. Reaction of a compound bearing hydroxyl groups with an inorganic acid as phosphoric or sulphuric acid or an acid derivative such as polyphosphoric acid, phosphorus pentoxide, phosphorus oxychloride, phosphorus acid, phosphorus trichloride, sulphur trioxide, halogenosulphonic acid, in the ab-

sence or presence of an inert solvent, to yield the corresponding acid ester.

e. Alkylation of phosphoric or phosphorus acid or their salts.

f. Reaction of aromatic polycarboxylic acids or their derivatives with a polyglycol at elevated temperature, with subsequent esterification of one of the free carboxylic acid groups with an aliphatic alcohol in the presence of catalyst.

h. Addition of alkylene oxide on inorganic carboxylic acids, amines, monovalent or multivalent alcohols in the presence of an alkaline catalyst, and subsequent reaction of the terminal hydroxyl groups with a halogen acid or an unsaturated  $\alpha,\beta$ -carboxylic acid, e.g. monochloracetic, acrylic, crotonic or methacrylic acid, in the presence of sodium hydroxide at elevated temperature.

i. Addition of epichlorohydrin on polyglycols at high temperature in the presence of a Lewis acid as catalyst, subsequent cleavage of hydrogen chloride by the addition of sodium hydroxide, reaction of the resulting diepoxide with ammonia or an amine, and finally alkylation with monochloracetic acid in aqueous solution with the addition of alkali.

The starting products named in the following can be 40 used to produce compounds conforming to this invention.

The carboxylic acids may be saturated or unsaturated, aliphatic or aromatic mono- or poly-carboxylic acids, preferably polycarboxylic and/or sulphocarboxylic acids, or their derivatives such as the anhydrides, esters or halides, notably the chlorides or bromides. Of the saturated dibasic acids may be named oxalic, malonic, succinic, adipic and azelaic acid; of the unsaturated dibasic acids maleic and fumaric acid; of the hydroxyl-substituted acids maleic, tartaric and citric acid; of the aromatic dicarboxylic acids phthalic, isophthalic and terephthalic acid; of the aromatic tricarboxylic acids trimellitic, hemimellitic and trimesic acid; of the aromatic tetracarboxylic acids mellophanic and pyromellitic acid; and as hexacarboxylic acid mellitic acid. Further, mention may be made of diphenyldicarboxylic acid, aliphatic and aromatic sulphocarboxylic acids, sulphuric acid esters such as sulphosuccinic and sulphotricarballylic acid, the sulphation products of fatty acids such as oleic acid, sulphuric acid esters of mono- and di-oxystearic acid, sulphobenzoic, sulphophenylacetic, sulphophenoxyacetic and sulphophthalic acids, sulphophthalic acid amides, naphthalenesulphonic and naphthalenopolysulphonic acids and their alkyl derivatives in which the alkyl chains bear one to 24 carbon atoms, alkane and alkene acids having preferably eight to 30 carbon atoms, for example caproic, caprylic, cyprie, lauric, myristic, stearic, arachic, be-

henic, oleic and ricinoleic acid, the corresponding sulphonic acids, the sulphates of the corresponding alcohols, aromatic monocarboxylic and monosulphonic acids such as phenolcarboxylic acids (salicylic acid), phenolsulphonic acids, their condensation products with formaldehyde, mono-, di- and tri-alkylphenolsulphonic acids, alkylphenylphosphoric acid esters such as amyl and diethyl derivatives, nonyl derivatives, dodecyl and octadecyl derivatives.

For esterification, saturated or unsaturated hydroxy compounds having preferably six to 30 carbon atoms are suitable, examples being octyl, lauryl, stearyl, behenyl, oleyl and bezyl alcohol, phenols, naphthols and their alkylation products, ethylene and propylene aducts from the aforesigned compounds which have one to 90, preferably one to 60, alkylene oxide units.

Of the polyglycols and copolymers of polyethylene and polypropylene oxide, the compounds having a molecular weight of about 200 to 6,000 deserve special mention.

To exemplify the starting materials used to form the organic derivatives of phosphoric or phosphorous acid, notably their esters from the corresponding alcohols or polyglycol derivatives, the following may be named: phosphoric and polyphosphoric acid, phosphorus pentoxide, phosphorus oxyhalides, phosphorus trihalides and phosphorous acid.

The suitable sulphonating agents include sulphuric acid, sulphur trioxide, chlorosulphonic acid, bisulphite and sulphur dioxide, in the presence of chlorine or oxygen.

The resins applied in conjunction with the disclosed compounds are preferably aminoplasts, which impart a crease resistant finish to textile substrates. As a rule, N-methylol urea or M-methylol melamine compounds can be used for this purpose with good success. Examples of formaldehyde and methylol resins of this type are the derivatives of compounds of formula



where  $A_1$  represents a radical of formula



and  $A_2$  represents hydrogen or lower alkyl. Other suitable resins are urea, melamines, e.g. tri-, tetra-, penta- and hexa-methylol melamine, carbamates, formaldehyde-acrolein and formaldehydeacetone condensation products, alkylolamides, e.g. methylol formamide, methylolacetamide, acrylamides, e.g. N-methylolformamide, N-methylolmetacrylamide, N-methylmethylolacrylamide, diureas, e.g. trimethylol and tetramethylol acetylene diurea, triazones e.g. dimethylol-N-ethyltriazone, haloacetamides, e.g. N-methylol-N-methylchloracetamide, urones, e.g. dimethylolurone and dihydroxydimethylolurone, and mixtures of these resins. The resin finishing of textiles is carried out preferably in the presence of catalysts. The salts of multivalent metals with strong mineral acids, ammonium and amine salts and acids are used as cata-

lysts for the reaction of N-methylol compounds. The suitable salts include the magnesium and zinc nitrates, phosphates and halides, zinc oxychloride, combinations of boric acid and calcium chloride, acetates, e.g. of zinc or magnesium. Ammonium sulphate, chloride and bromide are suitable ammonium salts; monoammonium and diammonium phosphate and alkanolamino hydrochlorides such as mono-, di- and triethanolamino hydrochloride can also be used.

- 10 Examples of suitable acids are hydrochloric, sulphuric and phosphoric acid, but preference is given to lower aliphatic acids such as propionic, glycolic, lactic, tartaric, citric and oxalic acid, and in particular formic or acetic acid, either alone or in combination with the

15 aforesigned metal salts. Also suitable are succinic, maleic, sulphuric and other acids. These acids can be used alone or in combination.

The compounds of this invention are applied to textile substrates in combination with a resin, preferably

20 one of the aforesigned N-methylol resins, and a catalyst. They are applicable to natural cellulosic (cotton, linen, hemp) and regenerated cellulosic fibres (viscose and cuprammonium rayon, polynosic and high wet modulus fibres), polyester, polyacrylonitrile, polypropylene, polyamide and other synthetic fibres, including blends of these fibres. They are of special interest for

25 finishing cotton and polyester textiles. The substrate may be present as loose fibre, yarn, woven or knit fabric, carpeting, felts or nonwovens, or in other textile

30 forms.

The compounds of formula (I) are applied to the high-polymer textile substrates in combination with optionally precondensed resins from aqueous-organic or preferably aqueous medium using the known methods.

- 35 It is preferable to employ the said compounds and resins in the form of preparations which may contain, for example, 10 to 90 percent of a compound of formula (I) and 10 to 90 percent resin, though the optimum ratio of the compound to the resin is 70:30 to 10:90.

40 Any of the standard methods of application is employable by means of which the preparations, if necessary after prior dilution, can be deposited on the substrate, for example padding, spraying, coating, dipping, printing, screen or foam application. It is desirable for the substrate to be finished with 0.01-10 percent or preferably 0.1-3 percent (relative to its weight) of the selected compound of formula (I) in combination with the resin. After intermediate drying (if necessary for the method used) the textiles are dry heat treated for fixation of the finish.

45

50

55 A suitable technique for applying the products of this invention jointly with N-methylol type resins is as follows. 50-300 or preferably 200-250 parts by weight of an approximately 50 percent aqueous solution of the N-methylol compound, which may if desired be partially condensed, are mixed with 20-300 or preferably 100-200 parts by weight of an almost neutral (pH—6-7), approximately 25 percent aqueous solution or dispersion of a compound of this invention, with the addition of 5-75 or preferably 20-30 parts by weight of one of the aforecited catalysts. The solution or dispersion is diluted to 1,000 parts with water. It is padded on fabric at 50°-150° C or preferably 80°-100° C and an expression giving an increase of 50-80 percent or preferably 70-75 percent on the dry weight, if necessary at reduced pressure or in an inert gas atmosphere. The fabric is treated in dry heat at 100°-220° C or preferably 120°-180° C for 1-10 or preferably 2-6 minutes to fix the finish, rinsed with water and dried.

The finish thus produced imparts durable soil repellency and crease resistance and greatly facilitates the removal of soil and oil in wash baths. Textile fabrics finished on these lines with products as disclosed herein have a soft handle, show a very good antistatic effect and, when dyed, undergo no loss or only minimal loss in the colour fastness properties.

In the following Examples, which illustrate the invention without limiting its scope, the parts and percentages are by weight and the temperatures in degrees centigrade. The products used in the Examples are specified in the preceding table.

1. General formula of the compounds listed in Table 1.



Table 1

| R'                                                              | R <sub>1</sub>                                                      | R <sub>2</sub>    | R <sub>3</sub> | E  | n    | Example |
|-----------------------------------------------------------------|---------------------------------------------------------------------|-------------------|----------------|----|------|---------|
| C <sub>18</sub> H <sub>35</sub>                                 | H                                                                   | COOH              | H              | 0  | 40   | 1       |
| C <sub>18</sub> H <sub>35</sub>                                 | H                                                                   | COOH              | COOH           | 0  | 40   | 1a      |
| C <sub>18</sub> H <sub>35</sub>                                 | H                                                                   | H                 | H              | 0  | 40   | 1b      |
| -C <sub>18</sub> H <sub>35</sub> C <sub>9</sub> H <sub>19</sub> | H                                                                   | COOH              | H              | 0  | 10   | 1c      |
| C <sub>18</sub> H <sub>35</sub>                                 | H                                                                   | H                 | H              | 0  | 25   | 1d      |
| C <sub>18</sub> H <sub>35</sub>                                 | H                                                                   | H                 | H              | 0  | 60   | 1e      |
| C <sub>6</sub> H <sub>5</sub>                                   | H                                                                   | H                 | H              | 0  | 10   | 1f      |
| C <sub>18</sub> H <sub>35</sub>                                 | H                                                                   | COOH              | COOH           | 0  | 25   | 1g      |
| H                                                               | C <sub>18</sub> H <sub>37</sub>                                     | COOH              | H              | 0  | 45   | 2       |
| H                                                               | C <sub>12</sub> H <sub>25</sub>                                     | COOH              | H              | 0  | 13.5 | 2a      |
| H                                                               | C <sub>17</sub> H <sub>35</sub> CONH(CH <sub>2</sub> ) <sub>2</sub> | COOH              | H              | 0  | 13.5 | 2b      |
| SO <sub>3</sub> H                                               | C <sub>18</sub> H <sub>37</sub>                                     | COOH              | H              | 0  | 13.5 | 3       |
| SO <sub>3</sub> H                                               | C <sub>18</sub> H <sub>37</sub>                                     | H                 | H              | 0  | 23   | 3a      |
| SO <sub>3</sub> H                                               | C <sub>18</sub> H <sub>37</sub>                                     | COOH              | H              | NH | 45   | 3b      |
| PO <sub>3</sub> H <sub>2</sub>                                  | C <sub>18</sub> H <sub>37</sub>                                     | COOH              | H              | 0  | 13.5 | 4       |
| PO <sub>3</sub> H <sub>2</sub>                                  | C <sub>18</sub> H <sub>37</sub>                                     | H                 | H              | 0  | 23   | 4a      |
| PO <sub>3</sub> H <sub>2</sub>                                  | C <sub>18</sub> H <sub>37</sub>                                     | COOH              | H              | NH | 45   | 4b      |
| C <sub>12</sub> H <sub>25</sub>                                 | H                                                                   | SO <sub>3</sub> H | H              | 0  | 0    | 11      |
| C <sub>18</sub> H <sub>37</sub>                                 | H                                                                   | SO <sub>3</sub> H | H              | 0  | )    | 11a     |
| C <sub>18</sub> H <sub>35</sub>                                 | H                                                                   | SO <sub>3</sub> H | H              | 0  | 25   | 11c     |
| C <sub>8</sub> H <sub>17</sub>                                  | H                                                                   | SO <sub>3</sub> H | H              | 0  | 0    | 11d     |



n = 25  
n = 40

Example 1h  
Example 1i



n = 23  
n = 13.5

R = C<sub>18</sub>H<sub>37</sub>  
R = C<sub>8</sub>H<sub>17</sub>

45



n = 45  
n = 23  
n = 13.5  
n = 6.5

Example 10  
Example 10a  
Example 10b  
Example 10c



n = 40 m = 1 R<sub>1</sub> = OH R<sub>2</sub> = COOH Example 6  
n = 25 m = 1 R<sub>1</sub> = OH R<sub>2</sub> = COOH Example 6a  
n = 40 m = 2 R<sub>1</sub> = H R<sub>2</sub> = H Example 6b  
n = 25 m = 2 R<sub>1</sub> = H R<sub>2</sub> = H Example 6c

55

38.4 Parts (0.2 mol) of trimellitic anhydride and 406 parts (0.2 mol) of oleylpolyglycol ether having 40 ethylene oxide groups are reacted for several hours at 150°-160° with stirring until the acid number reaches the value calculated for 0.4 equivalents. The trimellitic acid ester thus formed is a yellowish brown wax-like product. It dissolves readily in water and shows notably good soil repellent and antistatic properties.

Products with comparably good properties are obtained when, in place of trimellitic anhydride,

1a. pyromellitic dianhydride or  
1b. phthalic anhydride

are employed, or when in place of oleylpolyglycol ether with 40 ethylene oxide groups



65

|        |                                                                                  |                                                  |            |
|--------|----------------------------------------------------------------------------------|--------------------------------------------------|------------|
| n = 25 | R <sub>1</sub> = C <sub>18</sub> H <sub>35</sub>                                 | R <sub>2</sub> = H                               | Example 7  |
| n = 12 | R <sub>1</sub> = -C <sub>18</sub> H <sub>35</sub> C <sub>9</sub> H <sub>19</sub> | R <sub>2</sub> = H                               | Example 7a |
| n = 30 | R <sub>1</sub> = -C <sub>18</sub> H <sub>35</sub> C <sub>9</sub> H <sub>19</sub> | R <sub>2</sub> = H                               | Example 7b |
| n = 0  | R <sub>1</sub> = C <sub>18</sub> H <sub>37</sub>                                 | R <sub>2</sub> = C <sub>18</sub> H <sub>37</sub> | Example 12 |

5 6. R O(CH<sub>2</sub>CH<sub>2</sub>O)<sub>n</sub>CH<sub>2</sub>COONa

|                                        |          |            |
|----------------------------------------|----------|------------|
| R = C <sub>18</sub> H <sub>35</sub>    | n = 25   | Example 8  |
| R = C <sub>18</sub> H <sub>35</sub>    | n = 40   | Example 8a |
| R = C <sub>11</sub> H <sub>23</sub> CO | n = 6.8  | Example 8b |
| R = C <sub>11</sub> H <sub>23</sub> CO | n = 13.5 | Example 8c |
| R = C <sub>11</sub> H <sub>23</sub> CO | n = 23   | Example 8d |
| R = C <sub>17</sub> H <sub>35</sub> CO | n = 6.8  | Example 8e |
| R = C <sub>17</sub> H <sub>35</sub> CO | n = 13.5 | Example 8f |
| R = C <sub>17</sub> H <sub>35</sub> CO | n = 23   | Example 8g |



|                 |            |
|-----------------|------------|
| m + n + p = 15  | Example 9  |
| m + n + p = 60  | Example 9a |
| m + n + p = 120 | Example 9b |
| m + n + p = 9   | Example 9c |

- 1c. nonylphenylpolyglycol ether with 10 ethylene oxide groups,
- or in place of trimellitic anhydride and oleylpolyglycol ether with 40 ethylene oxide groups
- 1d. phthalic anhydride and oleylpolyglycol ether with 25 ethylene oxide groups;
- 1e. phthalic anhydride and phenylpolyglycol ether with 60 ethylene oxide groups,
- 1f. phthalic anhydride and phenylpolyglycol ether with 10 ethylene oxide groups,
- 1g. pyromellitic dianhydride and oleylpolyglycol ether with 25 ethylene oxide groups,
- 1h. pyromellitic dianhydride and oleylpolyglycol ether with 25 ethylene oxide groups in the molar ratio 1:2, or
- 1i. pyromellitic dianhydride and oleylpolyglycol ether with 40 ethylene oxide groups in the molar ratio 1:2.

#### EXAMPLE 2

192 Parts (1 mol) of trimellitic anhydride and 270 parts (1 mol) of stearyl alcohol are reacted at 150°-160° for several hours with stirring until the acid number reaches the value calculated for 2 equivalents. 231 Parts (0.5 mol) of the trimellitic acid stearyl ester thus formed are dissolved in 1,000 parts (0.5 mol) of polyethylene glycol, molecular weight 2,000, 0.5 part of concentrated sulphuric acid and 200 parts of xylene in a sulphonation vessel fitted with a water separator. The solution is brought to the boil with thorough stirring and boiled with reflux until no further water separates out and the acid number approximates to the calculated value. The solvent is then evaporated, leaving as residue the trimellitic acid diester. In the form of the sodium salt this product has good water solubility and is highly suitable for the soil repellent finishing of textiles.

Products of similarly good quality are obtained when the stearyl alcohol and polyglycol of molecular weight 2000 are replaced by

- 2a. lauryl alcohol and polyethylene glycol of molecular weight 600, or
- 2b. N-stearylaminooethyl alcohol and polyethylene glycol of molecular weight 600.

#### EXAMPLE 3

A solution of 192 parts (1 mol) of trimellitic anhydride, 270 parts (1 mol) of stearyl alcohol and 600 parts (1 mol) of polyethylene glycol, molecular weight 600, is reacted in analogy with the preceding Example. 104 Parts (0.1 mol) of the resulting trimellitic acid diester are dissolved in 200 parts of carbon tetrachloride, after which 23 parts (0.15 mol) of phosphorus oxychloride are added. The solution is held at 60° until the calculated amount of hydrogen chloride gas has escaped, upon which the solvent is evaporated and water added to hydrolyse the residue to the phosphoric acid ester. The product thus obtained is well soluble in water and is especially suitable for combined application with N-6 methylol compounds to produce durable soil and oil repellent finishes on textiles; these finishes impart a soft handle to the textiles and a very good antistatic effect. Moreover they have no adverse effect on the fastness properties of dyed goods.

Products with similarly good properties are obtained when in place of polyethylene glycol of molecular weight 600 and trimellitic anhydride

- 3a. polyethylene glycol (molecular weight 1000) and phthalic anhydride,
- or in place of stearyl alcohol and polyethylene glycol (molecular weight 600)
- 3b. stearyl amine and polyethylene glycol (molecular weight 2,000) are used.

#### EXAMPLE 4

104 Parts (0.1 mol) of the trimellitic acid diester obtained as intermediate in Example 3 are dissolved in 200 parts of carbon tetrachloride, with the subsequent dropwise addition of 11.7 parts (0.1 mol) of chlorosulphonic acid. The solution is maintained at 60° until the calculated amount of hydrogen chloride gas has escaped, then the solvent is evaporated. The sulphuric acid ester thus formed is well dispersible in water and is excellent for soil repellent finishing, having comparably good properties to the products obtained by the procedure of Example 3.

Further products with equally good properties can be produced by using in place of polyethylene glycol (molecular weight 600) and trimellitic anhydride

- 4a. polyethylene glycol (molecular weight 1,000) and phthalic anhydride
- or in place of stearyl alcohol and polyethylene glycol (molecular weight 600)
- 4b. stearyl amine and polyethylene glycol (molecular weight 2,000).

#### EXAMPLE 5

A solution of 296 parts (2 mols) of phthalic anhydride and 1,000 parts (1 mol) of polyethylene glycol, molecular weight 1,000, is held at 160°-180° until the acid number reaches the value calculated for 2 equivalents. A solution is prepared with 130 parts (0.1 mol) of the diphthalic acid ester thus formed, 27 parts (0.1 mol) of stearyl alcohol, 0.1 part of concentrated sulphuric acid and 80 parts of xylene. It is raised to the boil and held at this temperature long enough for the calculated amount of water to be distilled and the acid number to reach approximately the theoretical value. The solvent is then removed by distillation. A soft, wax-like product of beige colour is obtained when in the form of the sodium salt is readily soluble in water and shows particularly good soil repellent and antistatic properties.

In place of polyethylene glycol (molecular weight 1,000) and stearyl alcohol

- 5a. polyethylene glycol (molecular weight 600) and octanol can be employed, on which a product with comparable properties is formed.

#### EXAMPLE 6

A solution of 19.2 parts (0.1 mol) of citric acid, 203 parts (0.1 mol) of oleylpolyglycol ether with 40 ethylene oxide groups, 0.2 part of p-toluenesulphonic acid and 150 parts of xylene is set for reaction in a vessel equipped with stirrer and water separator. It is raised to the boil and held at this temperature until the acid number reaches the calculated value. After removal of the solvent by distillation, a pale, wax-like product of soft texture is obtained which is well soluble in water and is highly suitable for the soil repellent finishing of textiles.

Other products with comparable properties can be obtained by using in place of oleylpolyglycol ether with 40 ethylene oxide groups

- 6a. oleylpolyglycol ether with 25 ethylene oxide groups or in place of citric acid  
 6b. adipic acid  
 or in place of citric acid and oleylpolyglycol ether with 40 ethylene oxide groups  
 6c. adipic acid and oleylpolyglycol ether with 25 ethylene oxide groups.

## EXAMPLE 7

A solution of 19.2 parts (0.2 mol) of maleicanhydride and 274 parts (0.2 mol) of oleylpolyglycol ether with 25 ethylene oxide groups is reacted at 130°-150° until the acid number reaches the theoretical value. A solution of 25.2 parts (0.2 mol) of sodium sulphite in 100 ml of water is added, after which stirring is continued for 2 to 3 hours at 80°. The iodine consumption of a sample drops virtually to zero after this time. A 25 percent aqueous solution is obtained which has very good soil repellent and antistatic properties.

Products with equally good properties can be obtained by substituting for oleylpolyglycol ether with 25 ethylene oxide groups

- 7a. nonylphenylpolyglycol ether with 12 ethylene oxide groups or  
 7b. nonylphenylpolyglycol ether with 30 ethylene oxide groups.

## EXAMPLE 8

The solution for reaction is prepared with 137 parts (0.1 mol) of oleylpolyglycol ether having 25 ethylene oxide groups, 11.6 parts (0.1 mol) of the sodium salt of monochloracetic acid, 4 parts of sodium hydroxide, 0.16 part of sodium carbonate and 0.6 part of water. It is reacted for 5 hours at 100°, during which time the acid consumption of a sample decreases practically to zero. The product is readily soluble in water and has notably good power of soil repellency.

Other products showing comparable properties can be produced by using in place of oleylpolyglycol ether with 25 ethylene oxide groups

- 8a. oleylpolyglycol ether with 40 ethylene oxide groups,  
 8b. lauric acid polyglycol ester with 6.8 ethylene oxide groups,  
 8c. lauric acid polyglycol ester with 13.5 ethylene oxide groups,  
 8d. lauric acid polyglycol ester with 23 ethylene oxide groups,  
 8e. stearic acid polyglycol ester with 6.8 ethylene oxide groups,  
 8f. stearic acid polyglycol ester with 13.5 ethylene oxide groups,  
 8g. stearic acid polyglycol ester with 23 ethylene oxide groups.

## EXAMPLE 9

In analogy with Example 8, a solution of 150 parts (0.2 mol) of glycerotripolyglycol ether having three times 5 ethylene oxide groups, 70 parts (0.6 mol) of the sodium salt of monochloracetic acid, 24 parts (0.6 mol) of sodium hydroxide, 1 part of sodium carbonate and 5 parts of water is reacted to yield a yellowish product which is well soluble in water. It is highly suitable for the soil repellent and antistatic finishing of textiles.

Further products with similarly good properties are obtainable by using in place of glycerotripolyglycol ether containing three times 5 ethylene oxide groups,

- 9a. glycerotripolyglycol ether with three times 20 ethylene oxide groups or  
 9b. glycerotripolyglycol ether with three times 40 ethylene oxide groups.

## EXAMPLE 10

A solution of 500 parts (0.25 mol) of polyethylene glycol, molecular weight 2,000, 46.2 parts (0.5 mol) of epichlorohydrin and a small amount of borotrifluoroetherate is reacted in the known manner to form the dichlorohydrin ether. A solution of 20 parts (0.5 mol) of sodium hydroxide in 20 parts of water is added to convert the ether into the diepoxide. The separated sodium chloride is removed by filtration and the diepoxide dropped into 250 parts of 25 percent ammonia at room temperature for conversion into the diamine. When the end-point of the reaction is reached the batch is evaporated to dryness. A clear brownish product is obtained in a yield of 481 parts, its content of diamine (determined by filtration with perchloric acid) being approximately 70 percent.

A solution of 42.8 parts (0.02 mol) of the diamine, 4.7 parts (0.04 mol) of the sodium salt of monochloracetic acid, 1.6 parts of sodium hydroxide and 147.3 parts of water is reacted for several hours at about 80°, the reaction being terminated when the sulphuric acid consumption of a sample drops to nil. A clear pale yellow solution is obtained. The product is a very effective agent for the soil repellent finishing of textiles.

The polyethylene glycol of molecular weight 2,000 can be replaced by

- 10a. polyethylene glycol of molecular weight 1,000,  
 10b. polyethylene glycol of molecular weight 600 or  
 10c. polyethylene glycol of molecular weight 300; or again the molar ratio of the chosen polyethylene glycol of molecular weight 300-2,000 to the sodium salt of monochloracetic acid can be changed from 1:2 to a ratio between 1:4 and 1:6, upon which products with comparable properties are formed.

## EXAMPLE 11

A solution of 45.6 parts (0.2 mol) of 4-sulphophthalic anhydride-1,2 and 37.2 parts (0.2 mol) of dodecanol-1 is reacted for 3 hours at 130°, on which the acid number decreases to the theoretical value. The product thus formed is readily soluble in water. It gives very good service in the soil repellent finishing of textiles, without causing any loss in the fastness properties of disperse dyeings.

Other products exhibiting similarly good properties are obtained when the dodecanol-1 is replaced by

- 11a. stearyl alcohol or  
 11b. oleylpolyglycol ether with 25 ethylene oxide groups.

## EXAMPLE 12

A solution of 49 parts (0.5 mol) of maleic anhydride, 270 parts (0.1 mol) of stearyl alcohol, 0.5 part of p-toluenesulphonic acid as catalyst and 100 parts of toluene as decelerating agent is prepared in a sulphonation vessel fitted with a water separator. It is reacted for 5 hours at boiling temperature with reflux, during which time 8 millilitres of water is collected while the acid number decreases practically to zero.

A solution of 248 parts (0.4 mol) of the resulting maleic distearyl ester, 106 parts (0.416 mol) of a 41 per-

cent aqueous sodium hydrogen sulphite solution and 80 parts of methanol is reacted for 20 hours at 100° in an autoclave with stirring. Subsequently the remaining sodium hydrogen sulphite is decomposed with hydrogen peroxide. A white, well dispersible product is obtained. It is an excellent soil repellent agent for textiles and does not impair the fastness of disperse dyeings to any appreciable extent.

#### APPLICATION EXAMPLE A

A blend fabric of 67 percent polyester fibre and 35 percent cotton is padded with an aqueous dispersion containing 250 g/l of 50 percent aqueous dimethylol dihydroxyethyl urea, 25 g/l of  $Zn(NO_3)_2 \cdot 6H_2O$  and 200 g/l of the 25 percent aqueous (pH 6.5-7) product of Example 1, the expression on the padding machine giving a 75-80 percent increase on the dry weight. The fabric is dried at 120° and dry heat treated for 5 minutes at 160° for fixation of the finish. It is then cut into two halves. The first half is washed once and the second five times for 30 minutes at 60° with a commercial detergent. The two samples are then submitted to the tests described below.

##### a. Oil spotting test

The sample is spotted with used automobile oil, washed and assessed for ease of oil removal.

##### b. Soil deposition in washing

The sample is washed, dried and washed again in a wash bath set with 6 g/l of a fully active detergent and 5 g/l of an artificial soil mixture consisting of

|     |                      |
|-----|----------------------|
| 38  | % peat               |
| 17  | % cement             |
| 17  | % china clay         |
| 17  | % diatomaceous earth |
| 0.5 | % ferric oxide       |

20

A fabric of 67 percent polyester fibre and 33 percent cotton is padded at a liquor pickup of 75-85 percent with a liquor containing 250 g/l of 50 percent aqueous dimethylol propylene urea, 25 g/l magnesium chloride and 200 g/l of the 25 percent aqueous (pH 6.5-7) product of Example 10. The fabric is dried at 120° and the finish thermofixed for 5 minutes at 160°. It is then halved and the two samples tested as in Application Example A for soil repellency and soil deposition or greying in wash baths.

25 30 35 In the following table the test results are evaluated on a numerical scale from 1 to 5, where 5 represents excellent and 1 poor behaviour in the test. The two synthetic resins referred to in the first column of the table are dimethyl dihydroxy ethylene urea (I) and dimethylol propylene urea (II).

The degree of greying due to deposition of these impurities on the fabric in washing is assessed.

#### APPLICATION EXAMPLE B

A fabric of 67 percent polyester fibre and 33 percent cotton is padded at a liquor pickup of 75-85 percent with a liquor containing 250 g/l of 50 percent aqueous dimethylol methylcarbamate, 25 g/l of zinc chloride and 200 g/l of the 25 percent aqueous (pH 6.5-7) product of Example 4. After drying at 120° the finish is fixed by dry heat treatment for 5 minutes. The fabric is cut in two and the two samples tested for soil repellency and soil deposition in washing by the methods given in the preceding Application Example.

#### APPLICATION EXAMPLE C

A fabric of 67 percent polyester fibre and 33 percent cotton is padded at a liquor pickup of 75-85 percent with a liquor containing 250 g/l of 50 percent aqueous dimethylol propylene urea, 25 g/l magnesium chloride and 200 g/l of the 25 percent aqueous (pH 6.5-7) product of Example 10. The fabric is dried at 120° and the finish thermofixed for 5 minutes at 160°. It is then halved and the two samples tested as in Application Example A for soil repellency and soil deposition or greying in wash baths.

| Type of finish                                           | Oil spotting test |                   | Soil deposition in washing |                   | Fabric handle | Loss of fastness by disperse dyeings |
|----------------------------------------------------------|-------------------|-------------------|----------------------------|-------------------|---------------|--------------------------------------|
|                                                          | After one wash    | After five washes | After one wash             | After five washes |               |                                      |
| Synth. resin I + Prod. 1                                 | 3-4               | 3                 | 5                          | 2                 | soft          |                                      |
| Synth. resin I + Prod. 1a                                | 3                 | 3                 | 4                          | 2                 |               |                                      |
| Synth. resin I + Prod. 1b                                | 3-4               | 3                 | 5                          | 2                 |               |                                      |
| Synth. resin I + Prod. 1c                                | 3                 | 3                 | 4                          | 2                 |               |                                      |
| Synth. resin I + Prod. 1d                                | 3                 | 3                 | 4                          | 2                 |               |                                      |
| Synth. resin I + Prod. 1e                                | 3-4               | 3-4               | 4                          | 2                 |               |                                      |
| Synth. resin I + Prod. 1f                                | 3                 | 3                 | 3                          | 1                 |               |                                      |
| Synth. resin I + Prod. 1g                                | 3-4               | 3                 | 4                          | 2                 |               |                                      |
| Synth. resin I + Prod. 1h                                | 4                 | 3                 | 4                          | 2                 |               |                                      |
| Synth. resin I + Prod. 1i                                | 4                 | 4                 | 4                          | 3                 |               |                                      |
| Synth. resin I + Prod. 2                                 | 3                 | 3                 | 5                          | 3                 |               |                                      |
| Synth. resin I + Prod. 2a                                | 3-4               | 3-4               | 5                          | 2                 |               |                                      |
| Synth. resin I + Prod. 2b                                | 3                 | 3                 | 5                          | 2                 |               |                                      |
| Synth. resin I + Prod. 3                                 | 3-4               | 2-3               | 4                          | 2                 |               |                                      |
| Synth. resin I + Prod. 3a                                | 4                 | 3                 | 4                          | 2                 |               |                                      |
| Synth. resin I + Prod. 3b                                | 4                 | 3                 | 4                          | 3                 |               | slight                               |
| Synth. resin I + Prod. 4                                 | 3                 | 3                 | 5                          | 3                 |               | slight                               |
| Synth. resin I + Prod. 4a                                | 3-4               | 3                 | 5                          | 3                 |               | slight                               |
| Synth. resin I + Prod. 4b                                | 2-3               | 3                 | 4                          | 3                 |               | slight                               |
| Synth. resin I + Prod. 5                                 | 3                 | 3-4               | 4                          | 2                 |               |                                      |
| Synth. resin I + Prod. 5a                                | 3                 | 3                 | 4                          | 2                 |               |                                      |
| Synth. resin I + Prod. 6                                 | 3-4               | 4                 | 4                          | 3                 |               |                                      |
| Synth. resin I + Prod. 6a                                | 3-4               | 3                 | 3                          | 2                 |               |                                      |
| Synth. resin I + Prod. 6b                                | 4                 | 3-4               | 5                          | 3                 |               |                                      |
| Synth. resin I + Prod. 6c                                | 3                 | 3                 | 4                          | 2                 |               |                                      |
| Synth. resin I + Prod. 7                                 | 3-4               | 3                 | 4                          | 2                 |               |                                      |
| Synth. resin I + Prod. 7a                                | 3-4               | 3-4               | 4                          | 2                 |               |                                      |
| Synth. resin I + Prod. 7b                                | 3-4               | 3-4               | 4                          | 2                 |               |                                      |
| * Synth. resin I + alkylphenylpolyethylene glycol ether  | 3                 | 3                 | 1                          | 1                 | soft          | marked                               |
| Synth. resin I + polyacrylate product                    | 4                 | 3                 | 4                          | 1                 | stiff, harsh  |                                      |
| * Synth. resin I alone                                   | 3                 | 2                 | 1                          | 1                 | stiff, rough  |                                      |
| Synth. resin II + Prod. 1                                | 4                 | 2                 | 5                          | 3                 | soft          |                                      |
| Synth. resin II + Prod. 2                                | 4                 | 2                 | 4                          | 3                 | soft          |                                      |
| Synth. resin II + Prod. 2a                               | 4-5               | 2                 | 3                          | 2                 | soft          |                                      |
| Synth. resin II + Prod. 2b                               | 4                 | 2                 | 4                          | 3                 | soft          |                                      |
| * Synth. resin II + Alkylphenylpolyethylene glycol ether | 4-5               | 1-2               | 4                          | 2                 | soft          | marked                               |





where

R' is hydrogen or a saturated or unsaturated alkyl or aliphatic carboxylic acid radical which has one to 30 carbon atoms or a radical of an organic acid, E is oxygen or -NH-, R<sub>1</sub> is hydrogen or a saturated or unsaturated alkyl radical,

R<sub>2</sub> is hydrogen or a carboxyl or sulphoxyl group, R<sub>3</sub> is hydrogen or a carboxyl group, and n is zero or a value from one to 100.

10. A process according to claim 9 in which R' is alkyl of eight to 22 carbon atoms, E is oxygen, R<sub>1</sub> is hydrogen, R<sub>2</sub> is a sulphoxyl group,

R<sub>3</sub> is hydrogen or a carboxyl group, and n is zero or a value from one to 10.

11. A process according to claim 6 wherein in compound (c)

R is

